

## UNITED STATES PATENT OFFICE

1,957,494

## TREATMENT OF MATERIALS

George Holland Ellis, Spaldon, near Derby, England, assignor to Celanese Corporation of America, a corporation of Delaware

No Drawing. Application October 28, 1931,  
Serial No. 571,690. In Great Britain December  
20, 1930

12 Claims. (Cl. 8—5)

This invention relates to the production of pattern effects on textile materials and more particularly on materials made of or containing cellulose derivatives.

- 5 For the production of pattern effects on textile materials, the materials are commonly coloured with a ground colour, and then printed or otherwise locally treated with a composition which will discharge that colour in the printed areas; as an alternative, the material may first be printed with the discharge composition and then coloured with the ground colour, the printed areas remaining uncoloured. In both cases a dyestuff having an affinity for the material or capable of being fixed thereon, and which is resistant to the discharge may be incorporated in the discharge composition when coloured pattern effects upon a coloured ground may be obtained.
- 10 It is customary, after application of the discharge composition, to submit the materials to steaming or ageing or equivalent treatment in order to effect or complete the action of the discharging agent and also to fix properly colouring matter in the discharge preparation and/or the ground colour. In general a short steaming only is necessary to cause the discharging agent to act but a relatively much longer steaming for the fixation of the colour on the material. During the subsequent lengthy steam or equivalent after-treatment to fix the colour on the material there is a tendency for the discharging agent to suffuse into areas outside the printed areas so that the printed areas
- 15 become surrounded by "halos" or rings where the ground colour has become partially discharged or modified in shade. Such effects are especially liable to occur on materials made of or containing organic derivatives of cellulose as a somewhat prolonged steaming is in general necessary in producing pattern effects on these materials.

In producing discharge effects, particularly coloured discharge effects, upon textile materials in accordance with the present invention the foregoing defects due to suffusion of the discharging agent during steaming or equivalent after-treatment are avoided by counteracting the residual excess of discharging agent after discharge of the ground colour and before any

relatively lengthy ageing, steaming or like after-treatment requisite for the fixation of colouring matters applied in admixture with the discharging agent and/or for the purpose of ground colouration.

55 This counteraction, which further serves to prevent destruction of the illuminating colour during steaming or the like, is conveniently achieved by treating the material with a reagent opposite in character to the discharging agent; thus for example in the case of a reduction discharge the material may be treated with an oxidizing agent, or in the case of an oxidation discharge with a reducing agent.

60 The agents adapted to counteract the discharging agents may, after discharge of the ground colour, be applied to the materials in any convenient manner, for example in the form of aqueous solutions by padding. Thus a textile fabric may be uniformly coloured, then printed with a composition containing a reducing discharging agent and a dyestuff resistant thereto and having an affinity for the fabric, dried, aged, or steamed for a short time to effect the discharge of the ground colour in the printed areas, 75 then padded with a solution of an oxidizing agent, and finally subjected to steaming to fix on the material the dyestuff present in the discharge composition.

65 Examples of oxidizing agents suitable for counteracting excess of reducing discharging agents in accordance with the process of the present invention are bichromates, per-sulphates, and perborates. When employing acid reducing discharging agents such for example as stannous salts e. g. stannous chloride, it is of further advantage to incorporate an alkali with the oxidizing agent or to use an alkaline oxidizing agent. A very effective alkaline oxidizing agent is an alkali metal perborate.

80 The following examples illustrate in more detail the process according to the present invention, but it should be understood that these examples are given by way of illustration only and are in no way limitative:—

90 Example I

95 A fabric of cellulose acetate yarn, dyed a shade of Navy blue by diazotising ortho-methoxy-benzene-azo-alpha-naphthylamine on the material 100

and developing with betaoxynaphthoic acid, is printed with a paste of the following composition:—

|                                                                   | Grams |
|-------------------------------------------------------------------|-------|
| 5 1 - amino - 2 - methyl - anthraquinone 20% milled aqueous paste | 100   |
| Methylated spirits                                                | 100   |
| Gum arabic 1:1                                                    | 500   |
| Potassium sulphocyanide                                           | 25    |
| 10 Citric acid                                                    | 10    |
| Water                                                             | 115   |
| Stannous chloride                                                 | 150   |
|                                                                   | 1000  |

15 After drying and ageing the goods for a short time to effect the discharge of the ground colour they are padded with a 1% solution of sodium perborate, dried and steamed for 30 to 40 minutes and then again washed and treated and subjected to any other desired finishing operations. A clear orange discharge on a Navy blue ground results, the lengthy steaming permitting the anthraquinone dyestuff to become fully fixed on the fibre so that little colour is lost on washing and a relatively deeper colour is obtained with the same amount of dyestuff. At the same time the attendant danger of suffusion of the discharging agent from the printed areas into surrounding areas is eliminated.

30 *Example II*

A woven fabric of cellulose acetate yarn is dyed according to known methods with 1% of Malachite green crystals colour index No. 657. The 35 fabric is then dried and prepared for printing as usual.

By means of the usual type of two-colour printing machine, the following two printing pastes are applied:—

|                                                        | Grams  |
|--------------------------------------------------------|--------|
| (i) Dark British gum 30%                               | 537.5  |
| Citric acid                                            | 120.0  |
| Sodium chlorate                                        | 150.0  |
| 45 Caustic soda                                        | 22.5   |
| Potassium ferricyanide                                 | 20.0   |
| 1 - amino - 2-methyl-anthraquinone (20% aqueous paste) | 150.0  |
|                                                        | 1000.0 |
|                                                        | Grams  |
| (ii) Dark British gum 30%                              | 537.5  |
| Citric acid                                            | 120.0  |
| Sodium chlorate                                        | 150.0  |
| 55 Caustic soda                                        | 22.5   |
| Potassium ferricyanide                                 | 20.0   |
| 1 - acetyl - amino - anthraquinone (20% aqueous paste) | 150.0  |
|                                                        | 1000.0 |

60 After printing, the fabric is dried and aged for 5-8 minutes in the continuous Matther & Platt ager. It is then padded in a 2% solution of sodium bisulphite, dried and steamed  $\frac{3}{4}$  hour 65 either in a "cottage steamer" or continuous apparatus.

There results a yellow and orange two-colour discharge on a green ground, the impression being characterized by the clarity of the edges, and 70 the illuminating colours being well fixed and therefore of good fastness to wet processing.

As has been stated this invention is particularly valuable for fabrics made of or containing organic cellulose derivatives. Examples of such cellulose derivatives are esters of cellulose such as

cellulose acetate, cellulose formate, cellulose propionate and cellulose butyrate or ethers of cellulose such as methyl cellulose, ethyl cellulose and benzyl cellulose. The invention is, however valuable also for the production of pattern effects on mixed materials containing cellulose derivatives and other textile fibres, e. g. cotton, regenerated cellulose, silk, wool, or other textile fibres, or on materials containing these fibres and no cellulose derivative.

80 What I claim and desire to secure by Letters Patent is:—

1. Process for the production of coloured discharge effects on textile materials comprising an organic derivative of cellulose, comprising applying thereto a discharging agent in admixture with a colouring matter resistant thereto, ageing to effect discharge, rendering ineffective the excess discharging agent, and thereafter steaming to effect fixation of the resistant colouring matter.

90 2. Process for the production of coloured discharge effects on textile materials comprising cellulose acetate, comprising applying thereto a discharging agent in admixture with a colouring matter resistant thereto, ageing to effect discharge, rendering ineffective the excess discharging agent, and thereafter steaming to effect fixation of the resistant colouring matter.

95 3. In the production of pattern effects on textile materials by processes involving the application of reducing discharging agents followed by steaming to fix colouring matters present on said textile materials, rendering the residual discharging agent ineffective by means of an oxidizing agent after effecting the discharge but prior to at least part of the after-treatment.

100 4. In the production of pattern effects on textile materials comprising an organic derivative of cellulose by processes involving the application of reducing discharging agents followed by steaming to fix colouring matters present on said textile materials, rendering the residual discharging agent ineffective by means of an oxidizing agent after effecting discharge but prior to at least part of the after-treatment.

110 5. In the production of pattern effects on textile materials comprising cellulose acetate by processes involving the application of reducing discharging agents followed by steaming to fix colouring matters present on said textile materials, rendering the residual discharging agent ineffective by means of an oxidizing agent after effecting discharge but prior to at least part of the after-treatment.

115 6. In the production of pattern effects on textile materials comprising an organic derivative of cellulose by processes involving the application of reducing discharging agents followed by steaming to fix colouring matters present on said textile materials, rendering the residual discharging agent ineffective by means of an oxidizing agent selected from the group consisting of chromates, persulphates and perborates after effecting discharge but prior to at least part of the steaming.

125 7. In the production of pattern effects on textile materials comprising cellulose acetate by processes involving the application of reducing discharging agents followed by steaming to fix colouring matters present on said textile materials, rendering the residual discharging agent ineffective by means of an oxidizing agent selected from the group consisting of chromates, persulphates and perborates after effecting dis-

85

85

90

95

105

110

115

120

125

130

135

140

150

charge but prior to at least part of the steaming.

8. Process for the production of coloured discharge effects on textile materials comprising an organic derivative of cellulose, comprising applying thereto a discharging agent in admixture with a colouring matter resistant thereto, ageing to effect discharge, applying to the materials by padding an agent adapted to render the excess discharging agent ineffective, and thereafter 10 steaming to effect fixation of the colouring matter.

9. Process for the production of coloured discharge effects on textile materials comprising cellulose acetate, comprising applying there- 15 to a discharging agent in admixture with a colouring matter resistant thereto, ageing to effect discharge, applying to the mate- rials by padding an agent adapted to render the excess discharging agent ineffective, and 20 thereafter steaming to effect fixation of the col- curing matter.

10. In the production of pattern effects on textile materials by processes involving the ap-

plication of discharging agents followed by steaming to fix colouring matters present on said textile materials, rendering ineffective the residual discharging agent after effecting discharge but prior to at least part of such steaming.

11. In the production of pattern effects on textile materials comprising an organic derivative of cellulose by processes involving the application of discharging agents followed by steaming to fix coloring matters present on said tex- tile materials, rendering ineffective the residual discharging agent after effecting discharge but prior to at least part of such steaming.

12. In the production of pattern effects on textile materials comprising cellulose acetate by 90 processes involving the application of discharg- ing agents followed by steaming to fix coloring matters present on said textile materials, ren- dering ineffective the residual discharging agent 95 after effecting discharge but prior to at least part of such steaming.

GEORGE HOLLAND ELLIS.

26

100

30

105

40

110

45

115

50

120

55

125

60

130

65

135

70

140

75

150